

# United States Patent Office

3,250,637

Patented May 10, 1966

1

3,250,637

## HEAT STENCILIZABLE STENCIL

Paul E. Frasher, Chicago, Abraham D. Davis, Dolton, and Hersh A. Platkevich, Chicago, Ill., assignors to A. B. Dick Company, Niles, Ill., a corporation of Illinois  
No Drawing. Filed July 7, 1961, Ser. No. 122,423  
2 Claims. (Cl. 117—35.5)

The present invention relates to a stencil of the type having a coating thereon which will react when subjected to heat to provide an imaged area.

In Patent No. 2,808,777, issued to Allen I. Roshkind on October 8, 1957, there is described a system wherein a coating which is displaceable at temperatures of the order of 200° F. is provided on a fibrous backing. The coated sheet is adapted to be positioned adjacent an original which has outlines thereon capable of absorbing infra red radiation and generating heat in response thereto. Infra red rays are directed onto the assembly of the coated sheet and the original and the coating on the sheet is displaced to provide a stenciled image thereon. The coating is a relatively non-infra red ray absorbing material and is ink impervious. Therefore, when the stencil is placed on a duplicating machine ink will penetrate only in the stenciled image area and multiple copies may be produced.

The conventional materials employed for the displaceable coatings have been employed in relatively large amounts to provide a sufficiently strong stencil sheet. Furthermore, the thickness of standard stencil sheets of the thermographic type has been excessive due to the fact that the coating materials employed are not sufficiently abrasion resistant to permit the use of thinner coatings.

These attributes of prior stencils of the type described add to the cost of the items and it is therefore an object of this invention to provide a more economical and otherwise improved stencil of the thermographic type.

It is an additional object of this invention to provide a heat stencilizable stencil with a heat displaceable, ink impervious coating which need not be employed in relatively large amounts to provide a satisfactory stencil.

It is a further object of this invention to provide an improved thermographic stencil with a coating having the above noted properties and also having sufficient abrasion resistance whereby the use of thinner coatings is made possible.

These and other objects of this invention will appear hereinafter and it will be understood that the various examples hereinafter set forth are provided for purposes of illustration and not for purpose of limitation.

The heat stencilizable stencil of this invention is characterized by a light weight and thin base sheet having a coating composed of various amounts of a hard, high melting point wax, with or without paraffin wax, and wax soluble polymer additives.

The base sheet employed in the thermographic stencil of this invention comprises a sheet of thin, porous tissue having a weight from 4 to 7 pounds and preferably 4 to 5 pounds per 3,000 square feet of tissue. The tissue employed is a standard stencil base sheet insofar as composition is concerned, such as is formed of yoshino fiber, synthetic organic fiber or mixtures thereof, and it is preferably provided in thicknesses of from 0.8 to 1.2 mils, although thicknesses up to 2 mils are contemplated. The porosity, as measured on a Gurley Permeameter-4 ply, is preferably above 200 cu. ft./sq. ft./min.

The coating which is applied to the described tissue is composed of from 50 to 100% of a hard, high melting point wax. The melting point of the wax should fall within the range of 160 to 210° F., and preferably is 190 to 195° F. or 200 to 210° F. The hardness of the wax (100 gr./77°/5 sec.) (ASTM D1321-61T) preferably falls

2

within the range of 5 to 10, but may fall within the broader range of 0 to 20.

The coating may include from 0 to 50% of any commercial paraffin wax and is preferably formulated to contain from 10-35 percent by weight of the paraffin wax. Likewise a wax soluble polymer can be added to increase the toughness and oil resistance of the coating in an amount within the range of 0-5 percent by weight and preferably 1-4 percent by weight. Suitable polymers may be selected from the group consisting of the copolymers of vinyl acetate and vinyl stearate, the copolymers of ethylene and vinyl acetate, and the copolymers of ethylene and ethyl acrylate.

As suggested above, the coating can be formulated of the high melting point wax having the above described characteristics alone, and the wax should be coated on the tissue to obtain a weight of from 4 to 10 pounds per 3,000 square feet.

Further examples of a suitable coating are as follows:

|                                         | Percent |
|-----------------------------------------|---------|
| 190-195° Be Square wax (Bareco Wax Co.) | 70      |
| 130-132° paraffin                       | 27      |
| Dow resin X-3488.3                      | 3       |
| 100                                     |         |

### Example A

|                                           | Percent |
|-------------------------------------------|---------|
| 190-210° F. High M.P. wax (Be Square wax) | 65      |
| Paraffin wax                              | 31      |
| Vinyl acetate-vinyl stearate copolymer    | 4       |
| 100                                       |         |

### Example B

|                                           | Percent |
|-------------------------------------------|---------|
| 190-210° F. High M.P. wax (Be Square wax) | 65      |
| Paraffin wax                              | 31      |
| Vinyl acetate-vinyl stearate copolymer    | 4       |
| 100                                       |         |

This wax mixture should be coated on the tissue to obtain a weight between 4 to 10 pounds per 3,000 square feet.

As a specific example of the application of this invention to the formation of a stencil, a mixture of the foregoing Example A was dissolved in hot toluene (140-150° F.) at a solids content of 25%. The solution was coated onto a 4.5 lb. (24 x 36—500) stencil base tissue at a coating weight of 5 to 6 pounds per 3,000 square feet and then dried.

In use, the stencil is placed adjacent an original having infra red ray absorbing, heat generating outlines thereon, and the assembly is subjected to a source of infra red radiation. Upon directing of a sufficient quantity of radiations rich in infra red onto the original, a temperature rise from ambient temperature to a temperature in the range of from 140° F. to 210° F. is realized in the imaged portion of the original to provide a heat pattern. The coating composition in the corresponding areas on the stencil sheet is reduced to a flowable condition and displaced upon transfer of the heat pattern whereby openings in the stencil sheet are provided through which ink can flow. The original may be employed in the form of a separate sheet or it can be present as an image applied directly to the stencilizable sheet.

The heat stencilizable stencils of this invention are particularly suitable for use in conjunction with an assembly described and claimed in applicants' copending application entitled Assembly for Imaging Heat Stencilizable Stencils, Serial No. 122,587, filed July 7, 1961. The assembly described in the copending application generally comprises a top sheet of a relatively infra red transparent, poorly heat conductive shield; a protective, infra red transparent film located beneath the top sheet; and an infra red transparent, heat conductive film located adjacent the protective film. The stencil sheet of this invention is adapted to be fitted between the protective film and the heat conductive film, and the original will be located beneath the heat conductive film. Stencils produced with an assembly

of this type are particularly free of objectionable background and dust or dirt on the original or on the belt or plate of the device used for imaging the stencil is effectively avoided.

The above described stencil is characterized by the use of a thinner base sheet which permits the application of a lighter coating on the base sheet. It is appreciated by the art that thinner stencil sheets enable the ultimate production of better copy and the particular coating employed with the stencil of this invention permits the use of a thinner coating due to the hardness of the materials employed.

There has been described a simple, practical method of making multiple copies of any original which has outlines thereon which will convert radiant energy to heat energy.

It will be understood that various modifications may be made in the above described stencil which provide the characteristics of this invention without departing from the spirit thereof, particularly as defined in the following claims.

We claim:

1. A heat stencilizable stencil comprising a base sheet having a weight of 4 to 5 pounds per 3,000 square feet, a thickness of from 0.8 to 1.2 mils and a minimum porosity of 200 cu. ft./sq. ft./min., and a coating on said base sheet uniformly applied in amounts of from 4 to 10 pounds per 3,000 square feet, said coating consisting essentially of from 61 to 89% of a wax having a melting point from

160 to 210° F., and a hardness of from 5 to 10 (100 gr./77° F./5 sec.), from 10 to 35% of a paraffin wax and from 1 to 4% of a wax soluble polymer.

2. A stencilizable stencil comprising a base sheet having a weight of 4 to 7 pounds per 3,000 square feet, a thickness from 0.8 to 2.0 mils and a minimum porosity of 200 cu. ft./sq. ft./min., and a coating on said base sheet uniformly applied in amounts of from 4 to 10 pounds per 3,000 square feet, said coating consisting essentially of from 61% to 89% of a wax having a melting point from 160° to 210° F., and a hardness of from 5 to 10 (100 gr./77° F./5 sec.), from 10 to 35% of a paraffin wax and from 1 to 4% of a wax soluble polymer.

References Cited by the Examiner

UNITED STATES PATENTS

|           |         |                |       |          |
|-----------|---------|----------------|-------|----------|
| 1,168,223 | 1/1916  | Pembroke       | ----- | 117—35.5 |
| 2,756,161 | 7/1956  | Horii          | ----- | 117—35.5 |
| 2,808,777 | 10/1957 | Roshkind       | ----- | 117—158  |
| 2,858,236 | 10/1958 | Asselin et al. | ----- | 117—68   |
| 2,877,196 | 3/1959  | Reding         | ----- | 260—28.5 |
| 2,927,039 | 3/1960  | Vander Weel    | ----- | 117—36.7 |
| 2,999,765 | 9/1961  | Boenau         | ----- | 117—76   |
| 3,062,675 | 11/1962 | Shelffo        | ----- | 117—35.5 |

WILLIAM D. MARTIN, Primary Examiner.

JOSEPH B. SPENCER, Examiner.